

Nov. 7, 1944.

G. J. MORGAN

2,362,085

## METHOD OF HEATING OPEN-HEARTH FURNACE CHARGES

Filed April 13, 1942



INVENTOR  
GUY J. MORGAN,  
by his attorneys  
Stebbins and Blinks

Patented Nov. 7, 1944

2,362,085

# UNITED STATES PATENT OFFICE

2,362,085

## METHOD OF HEATING OPEN-HEARTH FURNACE CHARGES

Guy J. Morgan, Poland, Ohio

Application April 13, 1942, Serial No. 438,704

12 Claims. (Cl. 75—43)

This invention relates broadly to the manufacture of steel and, more particularly, to the heating of the charge in an open-hearth furnace.

Various types of fuels have been employed heretofore for heating open-hearth furnace charges. While gaseous fuel has been used principally, other types such as pulverized coal, fuel oil and tar have been utilized (The Making, Shaping and Treating of Steel, 5th edition, Camp and Francis, page 383). Single-jet burners delivering a mixture of steam and atomized oil have been utilized heretofore for firing open-hearth furnaces with fuel oil. These burners produced diverging flames which effected melting of the scrap initially charged into the furnace at a relatively slow rate from the exterior only of the pile. Attempts were made to increase the rate at which scrap could be melted by increasing the velocity of the combustible as delivered from the burner. This expedient, however, produced a condition of slight vacuum at the firing end of the furnace and excess pressure at the stack end even though the pressure at the center of the roof was .05 to .07" of water. This caused an inrush of cold air through the charging door wickets and any other openings at the firing end, pushing hot gases toward the back of the furnace. The resulting concentration of hot gases at the back of the furnace overheated the brick work of the roof and the high pressure at the stack end also contributed to this result by holding the hot gases against the roof.

In addition to the aforementioned objectionable conditions resulting from attempts to fire open-hearth furnaces with fuel oil, it has not been possible to change the character of the flame from the burner to suit it to the successive stages of the steel-making operation because, with the burners used heretofore, any such change required the laborious adjustment of heavy air valves and disrupted the entire setting of the furnace.

I have invented a novel method of heating an open-hearth furnace charge and a novel burner specially adapted therefor, whereby I am able to effect rapid melting of the scrap initially charged into the furnace, and modification of the flame to suit it to the successive stages of operation subsequent to the melting. In a preferred practice of the invention, I fire spaced, converging jets of a combustible such as a steam-oil mixture at relatively low velocity, and a central air jet at higher velocity adapted to produce an inductive effect upon the combustible jets, preventing substantial spreading of the flame whereby a sharp,

i. e., highly oxidizing flame results which is effective to oxidize and melt the scrap quickly. I also provide a simple and efficient burner capable of producing thorough atomization of steam and oil and adapted to deliver the converging combustible jets and the central air jet in such manner that the resulting flame impinges on a limited area of the surface of the scrap and thereby expedites the melting thereof. In addition to shortening the time required to melt the scrap, my invention produces more even distribution of the heat over the furnace roof, thereby reducing the temperature thereof and the rate of deterioration.

Other advantages and novel features of the invention will be pointed out in greater detail during the following complete description and explanation which refer to the accompanying drawing. In the drawing,

Figure 1 is a partial longitudinal section through an open-hearth furnace showing the application of my burner thereto;

Figure 2 is a view partly in side elevation and partly in section along a central longitudinal plane showing the burner to enlarged scale;

Figure 3 is an end view with a part in section; and

Figure 4 is an elevation of a detail.

Referring in detail to the drawing and, for the present, to Figure 1, my novel burner indicated generally at 10 is mounted in the fuel port 11 of an open-hearth furnace 12 having a bottom 13, roof 14, air inlet port 15 communicating with air uptakes 15a and charging doors 16. The burner may be supported in the port 11 by any suitable means (not shown) and has connections to suitable sources of a combustible mixture such as steam and oil, and compressed air. As indicated in the drawing, the burner is positioned to deliver a sharp, concentrated flame 17 impinging on a relatively small area of the surface of a pile of scrap 18 built up on the bottom 13, and on top of the limestone, if any, forming part of the charge.

Before proceeding with a further explanation of the method of my invention the structure of the burner itself will be described in detail by reference to Figures 2 through 4, since the construction of the burner determines to a large extent the procedure contemplated by my invention. The burner per se is claimed in my application Serial No. 488,975 divided herefrom.

As best shown in Figure 2, the burner 10 comprises a hollow cylindrical body 20. It may conveniently be formed from a length of pipe threaded at its ends to receive couplings 21 and 22. A

plug 23 is threaded into the coupling 21 and closes the forward end of the burner body. The plug 23 has a central air nozzle 24 and converging nozzles 25 spaced circumferentially thereof adapted to deliver jets of a combustible mixture such as steam and atomized oil. The inclination of the nozzles 25 is such that their axes intersect the axis of the nozzle 24 substantially at the point where the jets from the several nozzles impinge on the scrap piled in the furnace. The nozzles are of such length and diameter as to produce well defined, substantially linear jets of fluid when the latter is supplied thereto under suitable pressure.

Air is supplied to the nozzle 24 through an air tube 26 extending axially through the body 20 of the burner and having a nipple 27 welded to the extreme end thereof and threaded into the plug 23. The tube 26 extends through a plug 28 threaded into the coupling 22 and is connected to a suitable source of air under substantial pressure, e. g., 60-80# per square inch. The plug 28 is adapted to receive a packing gland 29 in its outer end and is provided with studs 30 whereby the gland may be drawn home around the air tube 26.

A combustible supply pipe 31 intersects the body 20 tangentially and at an acute angle to the projection of the axis of the body whereby atomized steam and oil delivered through the pipe 31 to the body are caused to travel forward therealong while circling about interiorly thereof. This insures thorough agitation and completes the mixing of the steam and oil and the atomization of the latter. The initial mixing of the steam and oil and atomization of the latter may be effected by any suitable means such as a simple form of steam-jet injector.

Having described the structure of the burner, it remains to explain the method which I practice by the aid thereof.

When the scrap has been completely charged through the doors 16, I supply a combustible mixture such as steam and oil through the pipe 31 and compressed air through tube 26 in such manner that on ignition, a sharp or oxidizing flame is projected from the burner onto the scrap pile, as indicated in the drawing at 17. The combustible mixture is preferably supplied under such pressure that combustion thereof will be substantially complete before striking the scrap pile. The air is delivered under sufficient pressure to impart to the jet discharged from the nozzle 24 a velocity somewhat greater than that of the jets of combustible, whereby the air stream by induction, draws the combustible radially inward of the flame, thereby preventing substantial spreading or diffusion and producing a sharp or oxidizing flame. As a result, a highly oxidizing "sting" of flame follows along the central air stream which is effective to burn a hole in the pile of scrap. The method of adjusting the air and combustible supply will be explained later. The air supplied through the nozzle 24 affords the primary air for combustion of the fuel, at the same time secondary air is supplied through the air inlet port 15. Because of the sharp or oxidizing character of the flame and the central "sting" or tongue in particular, the greater portion of the heat evolved by combustion is brought to bear on a relatively limited area of the surface of the scrap pile which is oxidized and the oxide melted in a relatively short time.

In addition to concentrating the flame, the air

jet from the nozzle 24 (the oxygen of which is eventually all consumed in the combustion of oil) also serves to remove the melted scrap progressively from the point where the flame impinges on the pile. As the scrap melts, the molten metal is blown aside by the air or oxidized, at least partially, and then blown away, exposing fresh surfaces of the piled scrap to the action of the burner flame. This progressive erosion of the surface of the pile quickly results in the formation of a hole in the pile into which the flame extends.

As the melting of the scrap proceeds in the manner indicated above, I increase the velocity of the air from nozzle 24 and combustible jets from the nozzles 25, thereby delivering a longer flame adapted to enter the hole formed in the pile by the initial melting and erosion of the surface thereof. The fuel discharged into the hole eroded in the pile blows through the pile, traversing the crevices between the adjacent masses of metal therein, and burns by surface combustion. This heats the pile throughout from the interior thereof with the result that the melting, when once initiated, proceeds rapidly to completion with the accumulation of a bath of molten metal on the bottom 13.

After the scrap has been wholly melted, I modify the flame produced by my burner, to adapt it to the succeeding stage of the operation of the furnace. I reduce the pressure of the air supplied through tube 26 and increase the rate of fuel supply so that the burner delivers a soft, hot, luminous flame. Such flame is well adapted for the working of the charge after the addition of the molten pig iron. Under these conditions, the air entering the inlet 15 furnishes the greater portion of the oxygen needed for combustion. For the working of the charge, the valves controlling the air entering the inlet port 15 are adjusted to give 2% excess oxygen in the stack gases when the maximum amount of fuel needed for working the charge is being supplied to the burner 10, the waste gas sample being taken after the scrap has been melted, the pig iron added and the bath is entirely covered by the slag. Even with the reduced velocity of the air jet, it is still effective to concentrate the burner flame on the bath, thereby tending to prevent over-heating of the roof.

With the valves controlling the air entering the inlet 15 adjusted as just described, the desired melting flame will result if the pressure on the air supplied to nozzle 24 is raised to from 60 to 80#/sq. in. and the fuel reduced sufficiently to sharpen the flame or make it strongly oxidizing.

I may further modify the flame after the charge has been fully worked, and convert it to a holding flame, if desired. I accomplish this by cutting off the air supply to the tube 26 and reducing the amount of the combustible delivered by the nozzles 25. The reduced amount of combustible is burned with the oxygen of the air entering the inlet port 15, producing a yellow, highly reducing flame which is well suited for holding the charge at tapping heat. This holding flame will not burn the brick work.

In a particular instance, I have found that a good working flame may be obtained if the air supplied to the tube 26 is under a pressure of from 10 to 20#/sq. in. For the holding flame, the fuel should be reduced so that no unburned combustible passes out of the stack end of the furnace.

It will be apparent that my invention is char-

acterized by numerous important advantages over prior methods of heating open-hearth furnace charges and burners therefor. The principal advantage is the reduction in the time required to melt the scrap. In a particular operation, including a large number of heavy charges, the time required to melt the scrap by my invention was less by more than an hour, on the average, than the time formerly required. This reduction in melting time has a direct relation to the output of steel per hour, the increase being actually 1.5 tons per hour in the example mentioned.

A further advantage of the invention is that a more nearly balanced condition of the pressure of the atmosphere in the furnace is obtained. The use of a burner having a plurality of fuel jets spaced circumferentially of a central air jet permits the fuel velocity to be reduced materially, (for instance, in the ratio of 1:9 in the burner disclosed) as compared to the burners previously used having a single fuel nozzle. In other words, my burner produces a positive pressure on the furnace gases at both the firing end and the stack end but the pressure at the stack end is much less than that created by the use of the burners previously installed. Because of the fact that the gas pressure in the furnace is nearly balanced and is positive at all points, short flames blow out through the wicket holes in all charging doors and all other openings so that no cold air can enter to disturb the balanced condition. As a result, the roof is heated to a substantially uniform temperature throughout its entire area without the occurrence of localized hot spots which cause accelerated deterioration of the brick work. In an actual furnace operation, careful measurements showed a reduction of 100° F. in the temperature of the furnace roof when practicing my invention, as compared to the previous practice on the same furnace.

The furnace roof is protected from excessive heating not only during the scrap-melting period but also during the working period because of the fact that the working flame, like the scrap-melting flame, is concentrated and is directed onto the bath so that the greater portion of the heat is absorbed by the latter and only a relatively small portion by the roof. This condition has a further desirable result in that it hastens the progress of events in the "shaping" or working of the charge.

The ability to modify the character of the flame discharged by the burner, to suit the several stages of the entire operation such as scrap melting, working, and holding, is, of course, an important advantage, particularly since it does not disturb the general setting of the furnace nor involve adjustment of the main air valves controlling the flow of in-going air through the regenerator checkers, the uptake and inlet port into the furnace. All that is necessary to vary the character of the flame is the proper adjustment of the amount of fuel and high-pressure air supplied to my burner. This may be accomplished by the aid of small valves which may be easily operated by hand.

The burner itself, furthermore, is effective, as pointed out above, to produce thorough mixture of the steam and fuel and atomization of the latter (oil or tar) by the steam with which it is entrained, thereby increasing the efficiency and completeness of combustion when mixed with the

primary and secondary air in the neighborhood of the nozzle end of the burner.

Although I have described and illustrated only a preferred practice and embodiment of my invention, it will be understood that changes in the procedure and construction disclosed herein may be made without departing from the spirit of the invention or the scope of the appended claims.

I claim:

10. 1. In a method of heating an open-hearth furnace charge, the steps including discharging toward a pile of scrap in the furnace, spaced jets of combustible converging substantially on said pile, at a velocity such that combustion is substantially complete on contact of the flame with the pile, supplying secondary air around said jets, and discharging a stream of compressed primary air centrally of said jets and at a velocity greater than that of said jets, thereby inducing the combustible in said jets radially inward to prevent substantial spreading of the flame and forming an oxidizing tongue concentrated on a limited area of the surface of the pile.
15. 2. In a method of heating an open-hearth furnace charge, the steps including discharging toward a pile of scrap in the furnace, spaced jets of combustible converging substantially on said pile, supplying secondary air around said jets, and delivering a stream of compressed primary air centrally of said jets and at a velocity greater than that of said jets, thereby inducing the combustible in said jets radially inward to prevent substantial spreading of the flame and forming an oxidizing tongue concentrated on a limited area of the surface of the pile which hastens the melting of the scrap.
20. 3. In a method of heating an open-hearth furnace charge, the steps including discharging toward a pile of scrap in the furnace, spaced jets of combustible, supplying secondary air around said jets, and delivering a stream of compressed primary air centrally of said jets and at a velocity greater than that of said jets, thereby inducing the combustible in said jets radially inward to prevent substantial spreading of the flame and forming an oxidizing tongue of flame concentrated on a limited area of the surface of the pile which hastens the melting of the scrap.
25. 4. In a method of heating an open-hearth furnace charge, the steps including discharging toward a pile of scrap in the furnace, spaced jets of combustible, supplying secondary air around said jets, and delivering a stream of compressed primary air centrally of said jets and at a velocity greater than that of said jets, thereby inducing the combustible in said jets radially inward to prevent substantial spreading of the flame and forming an oxidizing tongue of flame concentrated on a limited area of the surface of the pile which hastens the melting of the scrap.
30. 5. In a method of heating an open-hearth furnace charge, the steps including discharging toward a pile of scrap in the furnace, spaced jets of combustible, supplying secondary air around said jets, and delivering a stream of compressed primary air centrally of said jets and at a velocity greater than that of said jets, thereby inducing the combustible in said jets radially inward to prevent substantial spreading of the flame and forming an oxidizing tongue of flame concentrated on a limited area of the surface of the pile which hastens the melting of the scrap.
35. 6. In a method of heating an open-hearth furnace charge, the steps including discharging toward a pile of scrap in the furnace, spaced jets of combustible, and delivering a stream of compressed air centrally of said jets and at a velocity greater than that of said jets, thereby inducing the combustible in said jets radially inward to prevent substantial spreading of the flame and forming an oxidizing tongue of flame concentrated on a limited area of the surface of the pile which hastens the melting of the scrap.
40. 7. In a method of heating an open-hearth furnace charge, the steps including discharging toward a pile of scrap in the furnace, spaced jets of combustible, and delivering a stream of compressed air centrally of said jets and at a velocity greater than that of said jets, thereby inducing the combustible in said jets radially inward to prevent substantial spreading of the flame and forming an oxidizing tongue of flame concentrated on a limited area of the surface of the pile which hastens the melting of the scrap.
45. 8. In a method of heating an open-hearth furnace charge, the steps including discharging toward a pile of scrap in the furnace, spaced jets of combustible, and delivering a stream of compressed air centrally of said jets and at a velocity greater than that of said jets, thereby inducing the combustible in said jets radially inward to prevent substantial spreading of the flame and forming an oxidizing tongue of flame concentrated on a limited area of the surface of the pile which hastens the melting of the scrap.
50. 9. In a method of heating an open-hearth furnace charge, the steps including discharging toward a pile of scrap in the furnace, spaced jets of combustible, and delivering a stream of compressed air centrally of said jets and at a velocity greater than that of said jets, thereby inducing the combustible in said jets radially inward to prevent substantial spreading of the flame and forming an oxidizing tongue of flame concentrated on a limited area of the surface of the pile which hastens the melting of the scrap.
55. 10. In a method of heating an open-hearth furnace charge, the steps including discharging toward a pile of scrap in the furnace, spaced jets of combustible, and delivering a stream of compressed air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surfaces of the scrap to the heat of said flame.
60. 11. In a method of heating an open-hearth furnace charge, the steps including discharging toward a pile of scrap in the furnace, spaced jets of combustible, and delivering a stream of compressed air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surfaces of the scrap to the heat of said flame.
65. 12. In a method of heating an open-hearth furnace charge, the steps including discharging toward a pile of scrap in the furnace, spaced jets of combustible, and delivering a stream of compressed air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surfaces of the scrap to the heat of said flame.
70. 13. In a method of heating an open-hearth furnace charge, the steps including discharging toward a pile of scrap in the furnace, spaced jets of combustible, and delivering a stream of compressed air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surfaces of the scrap to the heat of said flame.
75. 14. In a method of heating an open-hearth furnace charge, the steps including discharging toward a pile of scrap in the furnace, spaced jets of combustible, and delivering a stream of compressed air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surfaces of the scrap to the heat of said flame.

ward a pile of scrap in the furnace, spaced jets of combustible converging substantially on said pile, and delivering a stream of compressed air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surfaces of the scrap to the heat of said flame.

7. In a method of heating an open-hearth furnace charge, the steps including discharging toward a pile of scrap in the furnace, spaced jets of combustible, at a velocity such that combustion is substantially complete on contact of the flame with the pile, and delivering a stream of compressed air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surface of the scrap to the heat of said flame.

8. In a method of heating an open-hearth furnace charge, the steps including discharging toward a pile of scrap in the furnace, spaced jets of combustible, supplying secondary air around said jets, and delivering a stream of compressed primary air centrally of said jets at a velocity sufficient to induce the combustible in said jets radially inward to prevent substantial spreading of the flame whereby it forms an oxidizing tongue of flame concentrated on a limited area of the surface of the pile which blows aside the resulting oxidized and liquefied metal thereby exposing fresh surfaces of the scrap to the heat of said flame.

9. In a method of heating an open-hearth furnace charge, the steps including discharging toward a pile of scrap in the furnace, spaced jets of combustible converging substantially on said pile, and delivering a stream of compressed primary air centrally of said jets, to induce the combustible thereof radially inward and prevent substantial spreading of the flame thereby effecting localized melting and the blowing of a hole into

the pile, permitting heating thereof from the interior, then when the scrap is melted, adjusting the air supply to convert the flame into a soft luminous flame effective on the bath for working the charge during the addition of the other components thereof.

10. In a method of heating an open-hearth furnace charge, the steps including discharging toward a pile of scrap in the furnace, spaced jets of combustible converging substantially on said pile, and delivering a stream of compressed primary air centrally of said jets, to induce the combustible thereof radially inward and prevent substantial spreading of the flame thereby effecting localized melting and the blowing of a hole into the pile, permitting heating thereof from the interior, then when the scrap is melted, adjusting the air supply to convert the flame to a soft luminous flame effective on the bath for working the charge during the addition of the other components thereof and finally terminating the supply of primary air to convert the flame to a highly reducing holding flame toward the end of the heat.

11. In a method of heating an open-hearth furnace charge, the steps including fusing and blowing a hole into a pile of scrap in the furnace by a sharp, oxidizing flame, discharging a jet of primary air centrally of said flame, adjusting the flame to heat the pile interiorly, then, when the scrap is melted, adjusting the air supply to convert the flame to a soft luminous flame effective on the bath for working the charge during the addition of other components.

12. In a method of heating an open-hearth furnace charge, the steps including fusing a small area on a pile of scrap in the furnace by a sharp, oxidizing flame, discharging a jet of compressed primary air centrally of said flame thereby blowing a hole into the pile, adjusting the flame to heat the pile interiorly, then, when the scrap is melted, adjusting the air supply to convert the flame to a soft luminous flame effective on the bath for working the charge during the addition of other components and finally converting the flame to a highly reducing flame effective on the bath for holding the charge toward the end of the heat.

GUY J. MORGAN.